# EUROPEAN PATENT SPECIFICATION

(11) **EP 2 252 680 B1**
(45) Date of publication and mention of the grant of the patent: **20.06.2012**
(21) Application number: 09719383.3
(22) Date of filing: 22.01.2009
(51) Int. Cl.: C11D 3/37

(54) **LAUNDRY TREATMENT COMPOSITION COMPRISING POLYMERIC LUBRICANTS**
WÄSCHEBEHANDLUNGSMITTEL MIT POLYMEREN GLEITMITTELN
COMPOSITION DE TRAITEMENT DE LESSIVE COMPORTANT DES LUBRIFIANTS POLYMÉRIQUES

(30) Priority: 14.03.2008 EP 08152740
(43) Date of publication of application: 24.11.2010
(73) Proprietor: Unilever PLC, London EC4Y 0DY (GB); Unilever N.V., 3013 AL Rotterdam (NL)
(72) Inventor: BATCHELOR, Stephen, Norman, Wirral, Merseyside CH63 3JW (GB); PARKER, Andrew, Philip, Wirral, Merseyside CH63 3JW (GB)
(74) Representative: Elliott, Peter William
(86) International application number: PCT/EP2009/050700
(87) International publication number: WO 2009/112298

(56) References cited:
- EP-A- 0 071 422
- WO-A-03/074644
- DE-A1- 1 900 002

## Description

### FIELD OF INVENTION

The present invention relates to wash added, fabric care compositions and methods for using the same during the wash cycle of a consumer laundry process.

### BACKGROUND

Coloured clothes are extremely popular with consumers. To remove dirt on washing, the clothes are vigorously agitated in water with a washing formulation. This process leads to damage on the surface of the clothes, which reduces their aesthetic appeal.

DE-A-1900002 discloses granular laundry detergent compositions comprising 17% surfactants, 30% tripolyphosphate and 20% polyethylene of 40-190 microns or 7100 microns or 3-150 microns, or 20% polypropylene of 1-700 microns.

EP-A-71422 discloses a powdered cleaning composition which comprises 100 parts by weight of a particulate polymeric material having an average particle size of from 8 to 110 microns; from 4 to 500 parts by weight of an inorganic salt; and from 4 to about 500 parts by weight of a fluid component.

EP 1 478 720 (Procter & Gamble) discloses the use of dispersible polyolefin waxes in detergent formulations with mean particle sizes from 5nm to 5 microns.

### SUMMARY OF INVENTION

We have found that using polyolefin particles larger than described in the prior art provide improved colour care. Further these larger polyolefin particles are easier to incorporate into a detergent composition because they do not need to be pre-dispersed before dosing.

In one aspect the present invention provides a granular laundry treatment composition containing less than 1 wt.% of phosphate comprising:
(i) from 0.2 wt.% to 4 wt.% of a polyolefin particle, the polyolefin particle having a size in the range from 25 to 5000 microns;
(ii) from 2 to 70 wt.% of a surfactant; and,
(iii) from 1 to 50 wt.% of a builder, wherein the builder comprises zeolite, wherein the polyolefin particle has a weight average molecular weight in excess of 2000, and has an acid number of from 0 to 200 mg/g KOH.

A second aspect of the invention provides a domestic method of treating a textile, the method comprising the steps of:
(i) treating a textile with an aqueous solution of from 1 to 20 g/l of the composition of the first aspect; and,
(ii) rinsing and drying the textile.

### DETAILED DESCRIPTION OF THE INVENTION

The amount of components in the granular laundry treatment composition quoted herein are wt.% of total composition unless otherwise stated.

The polyolefin particle should not dissolve in water or surfactant solutions. Such that when 1g/L of particles are placed into an aqueous solution containing 2g/L of sodium dodecyl sulphate at room temperature and shaken at 100 RPM on a rotator shaker at 293K for 2 hours, then removed from solution by filtering through a sieve or filter paper of appropriate size and dried. The weight of the particle removed is within 95 more preferably 99% of that added.

The polyolefin particle should have a weight average molecular weight in excess of 2000, preferably in excess of 10000. The weight average molecular weight may be measured by vapour phase osmometry or cryoscopy.

The polyolefin particle has an acid number from 0 to 200 mg/g KOH and preferably from 0 to 4 mg/g KOH (wherein the acid number indicates the mg of KOH needed to neutralize 1 g of polyolefin). Preferably the particles are spherical or elliptical in cross-section.

Preferably the particles are white, such that when their colour is measured using a reflectometer (UV excluded) and expressed as CIE L*a*b* values, L*>70, a* is between -3 and +3 and b^{*} is between 5 and -10.

The density of the particle is preferably 0.85 to 1.1 g/cm³, more preferably 0.95 Lo 1.05 g/cm³.

More preferably the polyolefin particle is selected from:
(a) polyethylenes:
(b) polypropylenes:

It is most preferred that the polyolefin particle is a polyethylene.

The size of the polyolefin particle is measured using graded sieves and it is that that is retained or passes through such sieves.

The polyolefin particle is sized preferably from 50 to 2500 microns.

An advantage over the disclosure of EP 1 478 720 is that the use of a larger particle size provides ease of incorporation of the polyolefin particle into the composition, i.e., the particle may be added directly rather than via a suspension, dispersion, or an emulsion of polyolefin wax. Thus the granular laundry treatment composition can be provided by post-dosed addition of polyolefin particles. Another advantage is that larger particles are much less likely to become airborne during handling or sniffing and consequently less likely to be inhaled.

### SURFACTANT

The composition comprises between 2 to 70 wt.% of a surfactant, most preferably 10 to 30 wt.%. In general, the nonionic and anionic surfactants of the surfactant system may be chosen from the surfactants described "Surface Active Agents" Vol. 1, by Schwartz & Perry, Interscience 1949, Vol. 2 by Schwartz, Perry & Berch, Interscience 1958, in the current edition of "McCutcheon's Emulsifiers and Detergents" published by Manufacturing Confectioners Company or in "Tenside-Taschenbuch", H. Stache, 2nd Edn., Carl Hauser Verlag, 1981. Preferably the surfactants used are saturated.

Suitable nonionic detergent compounds which may be used include, in particular, the reaction products of compounds having a hydrophobic group and a reactive hydrogen atom, for example, aliphatic alcohols, acids, amides or alkyl phenols with alkylene oxides, especially ethylene oxide either alone or with propylene oxide. Specific nonionic detergent compounds are C₆ to C₂₂ alkyl phenol-ethylene oxide condensates, generally 5 to 25 EO, i.e. 5 to 25 units of ethylene oxide per molecule, and the condensation products of aliphatic C₈ to C₁₈ primary or secondary linear or branched alcohols with ethylene oxide, generally 5 to 40 EO.

Suitable anionic detergent compounds which may be used are usually water-soluble alkali metal salts of organic sulphates and sulphonates having alkyl radicals containing from about 8 to about 22 carbon atoms, the term alkyl being used to include the alkyl portion of higher acyl radicals. Examples of suitable synthetic anionic detergent compounds are sodium and potassium alkyl sulphates, especially those obtained by sulphating higher C₈ to C₁₈ alcohols, produced for example from tallow or coconut oil, sodium and potassium alkyl C₉ to C₂₀ benzene sulphonates, particularly sodium linear secondary alkyl C₁₀ to C₁₅ benzene sulphonates; and sodium alkyl glyceryl ether sulphates, especially those ethers of the higher alcohols derived from tallow or coconut oil and synthetic alcohols derived from petroleum. The preferred anionic detergent compounds are sodium C₁₁ to C₁₅ alkyl benzene sulphonates and sodium C₁₂ to C₁₈ alkyl sulphates. Also applicable are surfactants such as those described in EP-A-328 177 (Unilever), which show resistance to salting-out, the alkyl polyglycoside surfactants described in EP-A-070 074, and alkyl monoglycosides.

Preferred surfactant systems are mixtures of anionic with nonionic detergent active materials, in particular the groups and examples of anionic and nonionic surfactants pointed out in EP-A-346 995 (Unilever). Especially preferred is surfactant system that is a mixture of an alkali metal salt of a C₁₆ to C₁₈ primary alcohol sulphate together with a C₁₂ to C₁₅ primary alcohol 3 to 7 EO ethoxylate.

The nonionic detergent is preferably present in amounts greater than 10%, e.g. 25 to 90 wt.% of the surfactant system. Anionic surfactants can be present for example in amounts in the range from about 5 wt.% to about 40 wt.% of the surfactant system.

### BUILDERS OR COMPLEXING AGENTS

The composition comprises from 1 to 50 wt.% of a builder, wherein the builder comprises zeolite.

Builder materials may be selected from 1) calcium sequestrant materials, 2) precipitating materials, 3) calcium ion-exchange materials and 4) mixtures thereof.

It is preferred that when an insoluble inorganic builder, e.g., zeolite, is used the size is in the range 0.1 to 10 microns (as measured by The Mastersizer 2000 particle size analyzer using laser diffraction ex Malvern™).

Examples of calcium sequestrant builder materials include alkali metal polyphosphates, such as sodium tripolyphosphate and organic sequestrants, such as ethylene diamine tetraacetic acid.

Examples of precipitating builder materials include sodium orthophosphate and sodium carbonate.

Examples of calcium ion-exchange builder materials include the various types of water-insoluble crystalline or amorphous aluminosilicates, of which zeolites are the best known representatives, e.g. zeolite A, zeolite B (also known as zeolite P), zeolite C, zeolite X, zeolite Y and also the zeolite P-type as described in EP-A-0,384,070.

The composition may also contain 0-50 wt.% of a builder or complexing agent such as ethylenediaminetetraacetic acid, diethylenetriamine-pentaacetic acid, alkyl- or alkenylsuccinic acid, nitrilotriacetic acid or the other builders mentioned below. Many builders are also bleach-stabilising agents by virtue of their ability to complex metal ions.

Carbonate (carbonate (including bicarbonate and sesquicarbonate) is a preferred additional builder.

The composition contain as builder a crystalline aluminosilicate, preferably an alkali metal aluminosilicate, more preferably a sodium aluminosilicate. This is typically present at a level of less than 15 wt.%. Aluminosilicates are materials having the general formula:

0.8-1.5 M₂O. Al₂O₃. 0.8-6 SiO₂

where M is a monovalent cation, preferably sodium. These materials contain some bound water and are required to have a calcium ion exchange capacity of at least 50 mg CaO/g. The preferred sodium aluminosilicates contain 1.5-3.5 SiO₂ units in the formula above. They can be prepared readily by reaction between sodium silicate and sodium aluminate, as amply described in the literature. The ratio of surfactants to aluminosilicate (where present) is preferably greater than 5:2, more preferably greater than 3:1.

Additionally to the aluminosilicate builders, phosphate builders may be used. In this art the term 'phosphate' embraces diphosphate, triphosphate, and phosphonate species. However, the formulation comprises less than 1 wt.% of such phosphate builders. Preferably the laundry detergent formulation is free from phosphate builders.

Other forms of builder include silicates, such as soluble silicates, metasilicates, layered silicates (e.g. SKS-6 from Hoechst).

We have also found that the presence of an inorganic builder in particular a zeolite, (insoluble inorganic particulates) contributes to the abrasion of fabrics under wash conditions. The use of the larger polyolefin particles ameliorate this problem.

### SHADING AGENT

The granular laundry treatment composition preferably comprises a blue or violet shading agent in the range from 0.0001 to 0.01 wt.%. The shading agents reduce the perception of damage to many coloured garments and increase whiteness of white garments.

The shading agents are preferably selected from blue and violet dyes of the solvent disperse basic, direct and acid type listed in the colour index (Society of Dyers and Colourists and American Association of Textile Chemists and Colorists 2002).

Preferably a direct violet or direct blue dyes is present. Preferably the dyes are bis-azo, tris-azo dyes or triphendioxazine dye. The carcinogenic benzidene based dyes are not preferred.

Bis-azo copper containing dyes such as direct violet 66 may be used.

The most preferred bis-azo dyes have the following structure: or wherein:
ring D and E may be independently naphthyl or phenyl as shown;
R₁ is selected from: hydrogen and C1-C4-alkyl, preferably hydrogen;
R₂ is selected from: hydrogen, Cl-C4-alkyl, substituted or unsubstituted phenyl and substituted or unsubstituted naphthyl, preferably phenyl;
R₃ and R₄ are independently selected from: hydrogen and C1-C4-alkyl, preferably hydrogen or methyl;
X and Y are independently selected from: hydrogen, C1-C4-alkyl and C1-C4-alkoxy; preferably the dye has X= methyl; and, Y = methoxy and n is 0, 1 or 2, preferably 1 or 2.

Preferred bis-azo dyes are direct violet 7, direct violet 9, direct violet 11, direct violet 26, direct violet 31, direct violet 35, direct violet 40, direct violet 41, direct violet 51, and direct violet 99.

Preferred solvent and disperse dyes, are selected from, mono-azo or anthraquinone dyes, most preferably, solvent violet 13, disperse violet 27 disperse violet 26, disperse violet 28, disperse violet 63 and disperse violet 77.

A preferred pigment is pigment violet 23.

### ENZYMES

The granular laundry treatment composition preferably comprises one or more enzymes which provide cleaning performance and/or fabric care benefits. Examples of suitable enzymes include, but are not limited to, hemicellulases, peroxidases, proteases, cellulases, xylanases, lipases, phospholipases, esterases, cutinases, pectinases, mannanases, pectate lyases, keratinases, reductases, oxidases, phenoloxidases,- lipoxygenases, ligninases, pullulanases, tannases, pentosanases, malanases, arabinosidases, hyaluronidase, chondroitinase, laccase, and amylases, or mixtures thereof. A typical combination is an enzyme cocktail that may comprise, for example, a protease and lipase in conjunction with amylase. When present in a cleaning composition, the aforementioned additional enzymes may be present at levels from about 0.00001 wt.% to about 2 wt.%, from about 0.0001 wt.% to about 1 wt.% or even from about 0.001 wt.% to about 0.5 wt.% enzyme protein by weight of the composition.

Preferred enzymes are cellulases.

### FLUORESCENT AGENT

The composition preferably comprises a fluorescent agent (optical brightener). Fluorescent agents are well known and many such fluorescent agents are available commercially. Usually, these fluorescent agents are supplied and used in the form of their alkali metal salts, for example, the sodium salts. The total amount of the fluorescent agent or agents used in the composition is generally from 0.005 to 2 wt.%, more preferably 0.01 to 0.1 wt.%. Preferred classes of fluorescer are: Di-styryl biphenyl compounds, e.g. Tinopal (Trade Mark) CBS-X, Di-amine stilbene di-sulphonic acid compounds, e.g. Tinopal DMS pure Xtra and Blankophor (Trade Mark) HRH, and Pyrazoline compounds, e.g. Blankophor SN. Preferred fluorescers are: sodium 2-(4-styryl-3-sulfophenyl)-2H-napthol[1,2-d]trazole, disodium 4,4'-bis{[(4-anilino-6-(N methyl-N-2 hydroxyethyl) amino 1,3,5-triazin-2-yl)]amino}stilbene-2-2' disulfonate, disodium 4,4'-bis{[(4-anilino-6-morpholino-1,3,5-triazin-2-yl)]amino} stilbene-2-2' disulfonate, and disodium 4,4'-bis(2-sulfoslyryl)biphenyl.

### PERFUME

Preferably the composition comprises a perfume. The perfume is preferably in the range from 0.001 to 3 wt.%, most preferably 0.1 to 1 wt.%. Many suitable examples of perfumes are provided in the CTFA (Cosmetic, Toiletry and Fragrance Association) 1992 International Buyers Guide, published by CFTA Publications and OPD 1993 Chemicals Buyers Directory 80th Annual Edition, published by Schnell Publishing Co.

It is commonplace for a plurality of perfume components to be present in a formulation. In the compositions of the present invention it is envisaged that there will be four or more, preferably five or more, more preferably six or more or even seven or more different perfume components.

In perfume mixtures preferably 15 to 25 wt.% are top notes. Top notes are defined by Poucher (Journal of the Society of Cosmetic Chemists 6(2):80 [1955]). Preferred top-notes are selected from citrus oils, linalool, linalyl acetate, lavender, dihydromyrcenol, rose oxide and cis-3-hexanol.

Perfume and top note may be used to cue the fabric care benefit of the invention.

It is preferred that the laundry treatment composition does not contain a peroxygen bleach, e.g., sodium percarbonate, sodium perborate, and peracid.

### POLYMERS

The composition may comprise one or more polymers. Examples are carboxymethylcellulose, poly(ethylene glycol), poly(vinyl alcohol), polycarboxylates such as polyacrylates, maleic/acrylic acid copolymers and lauryl methacrylate/acrylic acid copolymers.

Polymers present to prevent dye deposition, for example poly(vinylpyrrolidone), poly(vinylpyridine-N-oxide), and poly(vinylimidazole), are preferably absent from the formulation.

### Experimental

### Example 1

Three knitted cotton fabric swatches (20 by 20 cm) dyed with Vat Blue 4 were washed in a compartment of a Quickwash Plus ™ fabric testing system (SDL international). In a separate compartment equivalent knitted cotton swatches were placed, but these were dyes with Reactive Orange 16. The machine was filled with 3.5 litres of 26° French Hard water and 24.5 g of Persil Colour Powder (ex UK) a Las/Non-ionic surfactant powder built with zeolite and carbonate. To this was added 0.5g of antifoam. The wash took 15 minutes, and following this the machine was drained, spun, and then three 90 second rinses performed, draining and spinning after each. Following the wash the fabric was tumble dried. The procedure was repeated 5 times. The whole experiment was then repeated but with the addition of 1g/L of various additives.

Following the washes the reflectances of the VAT Blue cloths at 430nm and the Reactive Orange cloths at 650nm were measured on a Murakami Goniospectrophotometer with an incident angle of 65° and a measurement angle of 55°. The reflectance of the new cloths was 27.20 for the Vat Blue and 65.13 for the reactive Orange. The reflectance was compare to the reflectance of new unwashed fabric, and expressed as ΔR = |R(new) - R(washed)|. The ΔR (powder control) for Vat Blue was 6.06 and for Reactive Orange was 5.36. In the results the average ΔR between the blue and orange cloths is given to 1 decimal place.

The results are shown in table 1.

**Table 1**

| **Product** | **ΔR_{average}** |
|---|---|
| Powder Control | 5.7 |
| Licowax PE520P ex Clariant A low density polyethylene particle (particle size ~140µm)¹ | 3.3 |
| Licowax PE520GR ex Clariant A low density polyethylene particle (particle size ~2000µm) | 3.4 |
| Licowax PE520 Fine Grain ex Clariant A low density polyethylene particle (particle size ~170µm)¹ | 3.5 |
| Asensa CL101 ex Honeywell An oxidised polyethylene particle (particle size ~12µm) | 4.0 |
| Shamrock S386 N5T ex Shamrock technology A dispersible polyethylene (particle size ~4.9µm)¹ | 4.2 |
| Ceridust 3731 ex Clariant A high density polyethylene particle (particle size ~11µm) | 4.2 |

| | |
|---|---|
| ¹ particle size measured by SEM of commercial sample use in experiment. | |

The large organic polymer particles maintain the cloth closer to the new, as indicated by smaller ΔR_{average} values.

### Example 2

The experiment of example 1 was repeated using different levels of Licowax PE520P. The results are shown in the table below for the Vat Blue dyes cloth.

| **Licowax level** | **ΔR₄₃₀** |
|---|---|
| 0 * | 6.1 |
| 0.05 * | 4.9 |
| 0.1 * | 4.6 |
| 1 | 4.3 |

| | |
|---|---|
| * Denotes comparative examples | |

The polyethylene particles are effective across a wide range of dosages.

### Example 3

### Exemplary Granular Laundry Formulations A,B,C,D

| **Formulation** | **A *** | **B *** | **C *** | **D** |
|---|---|---|---|---|
| NaLAS | 15 | 20 | 10 | 14 |
| NI(7EO) | - | - | - | 10 |
| Na tripolyphosphate | - | 15 | - | - |
| Soap | - | - | - | 2 |
| Zeolite A24 | 7 | - | - | 17 |
| Sodium silicate | 5 | 4 | 5 | 1 |
| Sodium carbonate | 25 | 20 | 30 | 20 |
| Sodium sulphate | 40 | 33 | 40 | 22 |
| Carboxy methylcellulose | 0.2 | 0.3 | - | 0.5 |
| Sodium chloride | - | - | - | 5 |
| Lipase | 0.005 | 0.01 | - | 0.005 |
| Protease | 0.005 | 0.01 | - | 0.005 |
| Amylase | 0.001 | 0.003 | - | - |
| Cellulase | - | 0.003 | - | - |
| Fluorescer | 0.1 | 0.15 | 0.05 | 0.3 |
| Direct Violet 9 | 0.0002 | 0.00015 | - | 0.0001 |
| Solvent Violet 13 | - | 0.002 | - | 0.001 |
| Licowax PE520P | 0.1 | 0.5 | 0.5 | 0.5 |
| Sulfonated Zn Pthalocyanine photobleach | 0.002 | 0.004 | - | - |
| Water, impurities & minors | To 100 wt.% | To 100 wt.% | To 100 wt.% | To 100 wt.% |

| | | | | |
|---|---|---|---|---|
| * Denotes comparative examples | | | | |

Enzyme levels are given as percent pure enzyme. Levels of direct violet 9, solvent violet 13 and Sulfonated Zn Pthalocyanine photobleach are given as pure dye. NI(7EO) refers to R-(OCH₂CH₂)ₙOH, where R is an alkyl chain of C12 to C15, and n is 7.

The formulations are prepared by adding direct violet 9, acid violet 7 and the Sulfonated Zn Pthalocyanine photobleach into the slurry which is then spray dried. Alternatively, the dyes and photobleach may be added via post-dosed MgSO₄ granules.

The solvent violet 13 was dissolved in non-ionic surfactant (7E0) and granulated onto bentonite clay, to give a granule containing 0.2 wt.% dye. This was post-dosed to the formulation.

The Licowax PE520P particles were post dosed to the formulation.

## Claims

1. A granular laundry treatment composition containing less than 1 wt.% of phosphate comprising:
(i) from 0.2 wt % to 4 wt.% of a polyolefin particle, the polyolefin particle having a size in the range from 25 to 5000 microns;
(ii) from 2 to 70 wt.% of a surfactant; and,
(iii) from 1 to 50 wt.% of a builder, wherein the builder comprises zeolite,
wherein the polyolefin particle has a weight average molecular weight in excess of 2000, and has an acid number of from 0 to 200 mg/g KOH.

2. A granular laundry treatment composition according to claim 1, wherein the polyolefin particle has a size in the range from 50 to 2500 microns.

3. A granular laundry treatment composition according to claim 1 or claim 2, wherein the polyolefin particle is polyethylene.

4. A granular laundry treatment composition according to any preceding claim, wherein the polyolefin particle has been added to the laundry treatment composition as post dosed particles of polyolefin particle.

5. A granular laundry treatment composition according to any preceding claim, wherein the zeolite has a size in the range from 0.1 to 10 microns.

6. A granular laundry treatment composition according to any preceding claim, wherein the laundry treatment composition comprises a blue or violet shading agent in the range from 0.0001 to 0.01 wt.%.

7. A granular laundry treatment composition according to any preceding claim, wherein the laundry treatment composition comprises one or more enzymes, at a level of from 0.00001 wt.% to 2 wt.%, preferably the enzyme is a cellulase.

8. A domestic method of treating a textile, comprising the steps of:
(i) treating a textile with an aqueous solution of from 1 to 20 g/l of the composition of any one of claims 1 to 7; and,
(ii) rinsing and drying the textile.

## Patentansprüche

1. Körniges Wäschebehandlungsmittel, das weniger als 1 Gew.-% Phosphat enthält, umfassend:
(i) 0,2 Gew.-% bis 4 Gew.-% eines Polyolefinpartikels, wobei das Polyolefinpartikel eine Größe im Bereich von 250 bis 5000 Mikrometer hat;
(ii) 2 bis 70 Gew.-% eines Tensids und
(iii) 1 bis 50 Gew.-% eines Builders, wobei der Builder Zeolith umfasst,
wobei das Polyolefinpartikel ein gewichtsmittleres Molekulargewicht von über 2000 hat und eine Säurezahl von 0 bis 200 mg/g KOH hat.

2. Körniges Wäschebehandlungsmittel gemäß Anspruch 1, wobei das Polyolefinpartikel eine Größe im Bereich von 50 bis 2500 Mikrometer hat.

3. Körniges Wäschebehandlungsmittel gemäß Anspruch 1 oder Anspruch 2, wobei das Polyolefinpartikel Polyethylen ist.

4. Körniges Wäschebehandlungsmittel gemäß einem vorangehenden Anspruch, wobei das Polyolefinpartikel dem Wäschebehandlungsmittel als nachdosierte Partikel von Polyolefinpartikeln zugesetzt worden ist.

5. Körniges Wäschebehandlungsmittel gemäß einem vorangehenden Anspruch, wobei der Zeolith eine Größe im Bereich von 0,1 bis 10 Mikrometer hat.

6. Körniges Wäschebehandlungsmittel gemäß einem vorangehenden Anspruch, wobei das Wäschebehandlungsmittel ein blaues oder violettes Tönungsmittel im Bereich von 0,0001 bis 0,01 Gew.-% umfasst.

7. Körniges Wäschebehandlungsmittel gemäß einem vorangehenden Anspruch, wobei das Wäschebehandlungsmittel ein oder mehrere Enzyme in einer Konzentration von 0,00001 Gew.-% bis 2 Gew.-% umfasst, wobei das Enzym vorzugsweise Cellulase ist.

8. Haushaltsverfahren zur Behandlung einer Textilie, umfassend die Schritte:
(i) Behandeln einer Textilie mit einer wässrigen Lösung von 1 bis 20 g/l des Mittels gemäß einem der Ansprüche 1 bis 7 und
(ii) Spülen und Trocknen der Textilie.

## Revendications

1. Composition de traitement de lessive granulaire contenant moins de 1 % en poids de phosphate comportant :
(i) de 0,2 % en poids à 4 % en poids d'une particule de polyoléfine, la particule de polyoléfine ayant une taille dans la plage de 25 à 5 000 microns ;
(ii) de 2 à 70 % en poids d'un tensioactif ; et,
(iii) de 1 à 50 % en poids d'un adjuvant, l'adjuvant comprenant une zéolite,
dans laquelle la particule de polyoléfine a un poids moléculaire moyen en poids excédant 2 000, et a un indice d'acidité de 0 à 200 mg/g KOH.

2. Composition de traitement de lessive granulaire selon la revendication 1, dans laquelle la particule de polyoléfine a une taille dans la plage de 50 à 2 500 microns.

3. Composition de traitement de lessive granulaire selon la revendication 1 ou la revendication 2, dans laquelle la particule de polyoléfine est du polyéthylène.

4. Composition de traitement de lessive granulaire selon l'une quelconque des revendications précédentes, dans laquelle la particule de polyoléfine a été ajoutée à la composition de traitement de lessive sous la forme de particules post-dosées de particule de polyoléfine.

5. Composition de traitement de lessive granulaire selon l'une quelconque des revendications précédentes, dans laquelle la zéolite a une taille dans la plage de 0,1 à 10 microns.

6. Composition de traitement de lessive granulaire selon l'une quelconque des revendications précédentes, dans laquelle la composition de traitement de lessive comprend un agent de nuançage bleu ou violet dans la plage de 0,0001 à 0,01 % en poids.

7. Composition de traitement de lessive granulaire selon l'une quelconque des revendications précédentes, dans laquelle la composition de traitement de lessive comprend une ou plusieurs enzymes, à un niveau d'environ 0,00001 % en poids à environ 2 % en poids, l'enzyme étant de préférence une cellulase.

8. Procédé domestique de traitement d'un textile, comprenant les étapes consistant à
(i) traiter un textile avec une solution aqueuse de 1 à 20 g/l de la composition selon l'une quelconque des revendications 1 à 7 ; et,
(ii) rincer et sécher le textile.
